

# United States Patent

Honda et al.

[15] 3,661,629

[45] May 9, 1972

[54] **METHOD FOR THE PROCESSING OF SYNTHETIC FIBERS USED FOR REINFORCING RUBBER**

[72] Inventors: **Kyomi Honda; Koji Misaki**, both of Mihara, Japan

[73] Assignee: **Teijin Limited**, Osaka, Japan

[22] Filed: **Mar. 19, 1970**

[21] Appl. No.: **21,178**

[30] **Foreign Application Priority Data**

Apr. 1, 1969 Japan.....44/25017

[52] **U.S. Cl.**.....117/138.8 F, 117/47 A, 117/138.8 N, 117/139.5 F, 117/161 UF, 117/167

[51] **Int. Cl.**.....D06m 15/26, B32b 27/06

[58] **Field of Search** .....260/484 R; 106/295; 117/138.8 F, 138.8 N, 77, 139.5 F

[56] **References Cited**

## UNITED STATES PATENTS

|           |         |                      |             |
|-----------|---------|----------------------|-------------|
| 3,103,448 | 9/1963  | Ross.....            | 117/161 X   |
| 3,388,104 | 6/1968  | Crovatt.....         | 260/31.4 X  |
| 3,218,222 | 11/1965 | Skeen et al.....     | 117/138.8 N |
| 3,282,724 | 11/1966 | Atwell.....          | 117/138.8 N |
| 3,437,610 | 4/1969  | Moult .....          | 117/138.8 N |
| 3,443,986 | 5/1969  | Watanabe et al. .... | 117/138.8 N |
| 3,525,206 | 8/1970  | Hersh et al.....     | 117/138.8 N |

## FOREIGN PATENTS OR APPLICATIONS

682,354 3/1964 Canada.....117/138.8 N

*Primary Examiner*—William D. Martin

*Assistant Examiner*—Sadie L. Childs

*Attorney*—Richard A. Anderson and Roy H. Massengill

[ 57 ]

## ABSTRACT

A method for the treatment of synthetic fibers used for reinforcing rubber, featuring treatment of the synthetic fiber used for reinforcing rubber with a treating agent in which a nonionic surface active agent (abbreviated as X below) with the following general formula:



where A represents  $(\text{CH}_2)_7-\text{CH}=\text{CH}-\text{CH}_2$  or  $(\text{CH}_2)_{10+}$  R<sub>1</sub>, R<sub>2</sub> and R<sub>3</sub> represent hydrogen atoms, or  $-\text{CO}-\text{R}'_1$ ,  $-\text{CO}-\text{R}'_2$ , and  $-\text{CO}-\text{R}'_3$ ; R'<sub>1</sub>, R'<sub>2</sub> and R'<sub>3</sub> represent aliphatic hydrocarbons with carbon numbers of 1 to 22; p, q, and r represent the molar numbers of the ethylene oxide added and p+q+r is a positive integer=5 to 300; is combined with partially oxidized polyethylene with an average molecular weight of 500 to 10,000 (Abbreviated as Y below) in proportions within the limits of X=5 to 40, Y=0.1 to 3.0, and in which these components are combined with a lubricating agent and a surface active agent in addition to the aforesaid nonionic surface active agent X to give a total quantity of 100 weight percent.

4 Claims, No Drawings

## METHOD FOR THE PROCESSING OF SYNTHETIC FIBERS USED FOR REINFORCING RUBBER

### BACKGROUND OF THE INVENTION

The present invention pertains to a method for processing synthetic fibers that are used for reinforcing rubber.

The objectives of this invention are to prevent the reduction in the strength of synthetic fibers used for strengthening rubber during hot bonding treatment, by treating the synthetic fiber used for reinforcing rubber with a special processing agent to improve strength, and in addition, to improve adhesion, heat resistance and fatigue resistance in such fibers.

It is the usual practice, when synthetic fibers used for reinforcing rubber are mixed in with the rubber, to treat the compound with bonding agents and to accomplish heat treatment for the purpose of improving the adhesion between the fiber and the rubber.

In such cases, the synthetic fiber used for reinforcing rubber that has been so treated has the defect of a loss in its fatigue resistance.

It is well known that partially oxidized polyethylene has been used for the treatment of polyamide fibers as a means of meeting this problem in Japanese Pat. No. 1968-16667. The increase in strength that should be expected cannot be produced by applying the treatment only to the cord as in the process covered by that invention. It also has the deficiency of reducing the bonding strength and the fatigue resistance of the cord.

Further, the concurrent utilization in the heat treatment of synthetic fibers of partially oxidized polyethylene and the emulsifiers polyoxyethylene-(20)-lauryl ether or polyoxyethylene-(20)-lauryl ester is well known in U. S. Pat. No. 3,103,448. These processing agents do not increase the strength of the cord adequately and are undesirable because they also reduce the bonding properties and fatigue resistance of the cord.

As a result of studies intended to eliminate these defects, the writers arrived at the knowledge, which formed the basis for this invention, that the treatment of synthetic fiber for reinforcing rubber with partially oxidized polyethylene and a special emulsifier in a compound containing both in appropriate proportions would increase the strength of the fiber and would, in addition, increase its bonding with the rubber, heat resistance and resistance to fatigue.

### SUMMARY OF THE INVENTION

Specifically, the present invention is a method of treating synthetic cord used for reinforcing rubber which has as its special feature the combination of nonionic surface active agent (abbreviated as X below) having the following general formula:



In the above formula, A represents  $(\text{CH}_2)_7\text{CH} = \text{CH}-\text{CH}_2$  or  $(\text{CH}_2)_{10}$ .  $\text{R}_1$ ,  $\text{R}_2$ ,  $\text{R}_3$  represent hydrogen atoms or  $-\text{CO}-\text{R}'_1$ ,  $-\text{CO}-\text{R}'_2$ , or  $-\text{CO}-\text{R}'_3$ .  $\text{R}'_1$ ,  $\text{R}'_2$  and  $\text{R}'_3$  represent aliphatic hydrocarbons with carbon numbers of 1-22. Further  $p$ ,  $q$ , and  $r$  represent the molar numbers of the ethylene oxide added and  $p + q + r$  is a positive integer = 5 to 300, with partially oxidized polyethylene (abbreviated as Y below) having an average molecular weight of 500 to 10,000, within the limits, by weight percent, of the  $\text{X} = 5$  to 40,  $\text{Y} = 0.1$  to 3.0. This is

then treated with a processing agent comprising a lubricating agent and a surface active agent in addition to the above-identified nonionic surface active agent, X, to give a total quantity of 100 weight percent.

5 The form of the synthetic fiber used for reinforcing rubber as covered in the present invention may be (for example) tire cord, belt cord, fibers used in waterproofing or other industrial fibers.

The synthetic fiber used in the present invention, may be, 10 for example, a polyester, or a polyamide, etc.

In the process covered by the present invention, the treating agent covered by the present invention may be added to the fiber during any process from the spinning of the said rubber reinforcing fiber, up to the hot bonding treatment.

15 The values for  $p$ ,  $q$  and  $r$  for the nonionic surface active agent used in the present invention represent the total molar numbers for the ethylene oxide added. It is mandatory that  $p + q + r = 5$  to 300. It is possible to dramatically increase the strength of the rubber treated within these limits. Particularly

20 desirable results can be obtained within the limits of  $p + q + r = 10$  to 150. It is undesirable that the total be less than  $p + q + r = 5$  as this reduces the bonding strength of the treated cord. It is also undesirable that the total be more than  $p + q + r = 300$  as this makes emulsification difficult and the cord which is treated becomes stiff and loses strength.

25 In the nonionic surface active agent covered by the present invention,  $\text{R}_1$ ,  $\text{R}_2$  and  $\text{R}_3$ , represent aliphatic hydrocarbons with carbon numbers of 1 to 22. The presence or absence of branched chains or double bonds is irrelevant. No exceptional

30 difference is observed in improving the strengthening effects of the synthetic fiber used for reinforcing rubber within the above described limits for aliphatic hydrocarbons with carbon numbers of more than 22, but emulsifiability is lost and the compound cannot be put to practical use. Carbon numbers of 8 to 17 are desirable in the aliphatic hydrocarbon from the viewpoint of the emulsifiability and the solubility of the processing compound.

35 It is possible to use only the nonionic surface active agent in the present invention and still increase the strength of the synthetic fiber used for reinforcing rubber. In such cases, however, it is necessary to increase the proportions of this agent within the treating compound to more than 80 weight percent in order to achieve the desired increase in strength. It is not

40 desirable to do so since this reduces bonding strength. This also has a markedly deleterious effect on the spinnability when it is utilized as a spinning oil in spinning. It can also not be used industrially owing to the extreme difficulties engendered in dissolution or emulsifying when it is used in an aqueous emulsion.

45 As a result of the utilization of the partially oxidized polyethylene and the nonionic surface active agent in the optimum proportions as covered in the present invention, it has been possible to overcome these obstacles and to increase dramatically the bonding properties and fatigue resistance during the strengthening of the treated cord.

50 It is mandatory that the partially oxidized wax utilized in the present invention be a partially oxidized polyethylene type wax with an average molecular weight of 500 to 10,100.

55 It is desirable that the acid value of the partially oxidized wax be 10 to 30, and that the softening point be below 125°C.

The commercial, partially oxidized waxes which fulfill these conditions are the partially oxidized microcrystalline waxes, for example, Petrolite C-5, C-23, C-36, PE 100 and Petronau-ba C, D, F, H and W, etc. The partially oxidized polyethylene waxes may be, for example, Hexto Wax Pead 521, Hexto Wax V P-522, Ebolene E and AC-655, etc.

60 It is necessary to add a lubricating agent and a surface active agent in addition to the nonionic surface active agent, X, to the previously described effective components in the processing agent used in the present invention. So long as the composition is maintained within the limits components X and Y, where  $\text{X} = 5$  to 40 weight percent and  $\text{Y} = 0.1$  to 3.0 weight percent, the lubricating agent and the surface active agent do

65

70

75

not interfere with the cord strengthening effects of the processing agent. The smoothing agent and the surface active agent may be added to component X and Y in quantities that will make the total quantity of the compound 100 percent.

The lubricating agent in the present invention may be mineral oil, a higher aliphatic alcohol ester or a vegetable oil, etc. The active agent which can be used together with these substances may be a nonionic surface active agent, except for the nonionic surface active agent X, for example, an addition compound of a higher alcohol and ethylene oxide. The ionic type surface active agent that may be used are, for example, a sulfuric acid ester salt, a phosphoric acid ester salt, etc. These lubricating agents and surface active agent improve the emulsifiability, the solubility and the smoothness of the processing agent and facilitate the spinning process and the cord manufacturing process.

In the process covered by the present invention, the treating agent may be applied to the synthetic fiber used for reinforcing rubber at any time from its spinning up to the heat bonding process by immersion, spraying, or any other suitable method for applying a thin coating to the fiber. The treating agent may be applied to the fiber as is, but it may also be used in a form of an aqueous emulsion or be dissolved in a solvent.

Fully adequate effects may be attained by applying the treating agent in quantities of 0.01 to 2.00 weight percent to the fiber being treated.

In the present invention, as a result of treating synthetic fiber used for reinforcing rubber with a treating agent composed of the special nonionic surface active agent X, and partially oxidized polyethylene Y, in quantities that lie within the limits X = 5 to 40 weight percent, Y = 0.1 to 3.0 weight percent, and a mineral oil and a surface (except for the above stated X), in quantities that will give a total weight percent of 100, in small quantities, make it possible to greatly increase the cord strength, its adhesion and its resistance to fatigue subsequent to bonding heat treatment. It is possible to improve spinnability by utilizing the treating agent covered by the present invention by using it as a spinning oil or a stretching oil during spinning and stretching.

The treatment covered by the present invention is particularly advantageous when used with polyamide fibers or polyester fibers that are used in tire cord.

#### DESCRIPTION OF THE PREFERRED EMBODIMENTS

##### Example 1

1680 denier nylon-6 (polycaproamide) cord formed of two 840 denier ends, 47 filaments per end was washed and

TABLE 1  
[Method covered by the present invention]

| Composition of the processing agents           | Test number |      |      |      |      |      |      |       |      |      |      |      |      |      |      | blank |
|------------------------------------------------|-------------|------|------|------|------|------|------|-------|------|------|------|------|------|------|------|-------|
|                                                | 1           | 2    | 3    | 4    | 5    | 6    | 7    | 8     | 9    | 10   | 11   | 12   | 13   | 14   | 15   |       |
| Partially oxidized polyethylene Y:             |             |      |      |      |      |      |      |       |      |      |      |      |      |      |      |       |
| Compound A                                     |             |      |      |      |      |      |      |       |      |      |      |      |      |      |      |       |
| Compound B                                     | 0.1         | 0.1  | 2.0  |      | 3.0  | 3.0  |      | 0.1   | 0.05 | 2.0  | 2.0  | 4.0  | 4.0  | 3.0  |      |       |
| Compound C                                     |             |      |      |      |      |      |      |       |      |      |      |      |      |      |      |       |
| Nonionic surface active agent X:               |             |      |      |      |      |      |      |       |      |      |      |      |      |      |      |       |
| Compound D                                     | 5.0         | 40.0 | 20.0 |      |      |      |      | 3.0   | 40.0 | 3.0  | 45.0 |      |      |      |      | 30.0  |
| Compound E                                     |             |      |      |      |      |      |      | 40.0  |      |      |      |      |      |      |      |       |
| Compound F                                     |             |      |      |      |      |      |      | 3.0   | 40.0 |      |      |      |      |      |      | 30.0  |
| Lubricating agent:                             |             |      |      |      |      |      |      |       |      |      |      |      |      |      |      |       |
| Mineral oil, Redwood viscosity at—             |             |      |      |      |      |      |      |       |      |      |      |      |      |      |      |       |
| 30° C., 60 sec.                                | 70.0        | 40.0 | 50.0 |      |      |      |      | 70.0  | 40.0 | 70.0 | 30.0 |      |      |      |      |       |
| 30° C., 150 sec.                               |             |      |      |      |      |      |      | 72.0  | 40.0 | 40.0 |      |      |      |      |      | 67.0  |
| Surface active agent:                          |             |      |      |      |      |      |      |       |      |      |      |      |      |      |      | 30.0  |
| Higher alcohol ethylene oxide addition product | 24.9        | 10.9 | 28.0 | 22.0 | 17.0 | 17.0 | 26.9 | 19.95 | 25.0 | 23.0 | 21.0 | 21.0 | 30.0 | 40.0 | 30.0 |       |
| Alkyl sulfate                                  |             |      |      |      |      |      |      |       |      |      |      |      |      |      |      | 10.0  |
| Cord properties:                               |             |      |      |      |      |      |      |       |      |      |      |      |      |      |      |       |
| Untreated cord strength, kg.                   | 15.0        | 15.0 | 15.0 | 15.0 | 15.0 | 15.0 | 15.0 | 15.0  | 15.0 | 15.0 | 15.0 | 15.0 | 15.0 | 15.0 | 15.0 |       |
| Treated cord strength, kg.                     | 15.1        | 15.2 | 15.6 | 15.2 | 15.6 | 15.5 | 14.5 | 14.5  | 14.6 | 15.5 | 15.3 | 15.5 | 14.8 | 14.0 | 14.3 | 14.0  |
| Bonding strength, kg.                          | 14          | 13   | 14   | 14   | 13   | 13   | 14   | 13    | 13   | 12   | 13   | 11   | 13   | 11   | 14   | 11    |
| Fatigue resistance, percent                    | 115         | 130  | 150  | 140  | 130  | 130  | 110  | 120   | 120  | 80   | 80   | 80   | 80   | 100  | 100  |       |

##### Explanation of Table 1

In the foregoing table, Compounds A-F represented the following:  
 Compound A=Vp-5001 (Hexto Company) acid value 15, softening point 97° C.  
 Compound B=Ebolen E (Eastman Company) acid value 10, softening point 105° C., specific gravity 0.94.  
 Compound C=AC-655 (Allied Chemical Company) acid value 15, softening point 104° C., specific gravity 0.93.  
 Compound D represented by the following formula:

70  
75



degreased. This cord was then immersed in a 2 percent aqueous emulsion of a treating agent having the various compositions shown in Table 1 as tests 1-15 and the blank test. After applying 0.5 weight percent of the treating agent to the cord, 8 percent of the below described bonding agent was applied to the cord, the cord was strengthened by hot bonding under a 12 percent stretch at 200° C. for 20 minutes. The measurement results for adhesion and resistance to fatigue were as given in Table 1. The measurements of resistance to fatigue were made by the Goodyear Fatigue Test, JIS L 1017-1963.

Adhesion was tested by the Hobverse side pulling test. The bonding agent used during the bonding treatment had the following composition:

#### Bonding Agent Composition

|                                               |                |
|-----------------------------------------------|----------------|
| Water                                         | 47.20%         |
| Caustic soda (10%)                            | 1.12%          |
| Ammonia (28%)                                 | 3.09%          |
| Adha-RF (Solid components 45.1%) <sup>1</sup> | 6.23%          |
| Nippon Zeon "LX-102" <sup>2</sup>             | 21.92%         |
| Nippon Zeon "Hycar 2508 FS" <sup>3</sup>      | 17.54%         |
| Formaldehyde (36.5%)                          | 2.90%          |
| <b>TOTAL</b>                                  | <b>100.00%</b> |

<sup>1</sup>condensation product of formaldehyde and resolin

<sup>2</sup>styrene-butadiene copolymer

<sup>3</sup>styrene-butadiene-vinylpyridine ter-polymer

As is clear from the results shown in the Table 1, the treating agent containing components X and Y within the compositional limits covered by the present invention, as when used in Tests No. 1-6 produced the result of raising the strength, adhesion and fatigue resistance of the cord subsequent to hot bonding treatment.

In contrast, there is an undesirable reduction in cord strength in Tests 7 and 9 (when there is insufficient component X) and in Test No. 8 when there is insufficient Y.

Further, in Tests 10 (when an excessive quantity of component X is used), Test 11 (when an excessive quantity of Y is used), and Test 12 (when there is an excessive quantity of both the X and Y components,) the strength of the cord is increased; however, there is an undesirable drop in adhesion and fatigue resistance.

The results in Tests 13 (when only component Y is used) are also undesirable since the strength of the cord is not raised sufficiently and the fatigue resistance drops.

Compound E = Same formula



In contrast, in the comparative examples (Tests No. 2 and 3) only the adhesion is raised. The strength of the treated cord is reduced and absolutely no increase in fatigue resistance can be observed, since the nonionic surface active agent used differed from that covered by the present invention, giving undesirable results.

### Example 3

A treating agent with the composition shown below was applied to nylon tire cord—as the first paragraph of the examples.

Ebolene E, Eastmen Company, partially oxidized polyethylene,

Ebolene E, Eastmen Company, partially oxidized polyethylene,

|                                                                                                                                                                                                                                       |                |
|---------------------------------------------------------------------------------------------------------------------------------------------------------------------------------------------------------------------------------------|----------------|
| Ebolene E, Eastman Company, partially oxidized polyethylene, acid value 10, specific gravity 0.94, softening point 105° C.                                                                                                            | Percent weight |
| $\begin{array}{c} \text{CH}_2-\text{O}-\text{CO}-\text{(CH}_2\text{)}_{10}-\text{CH}-\text{(CH}_2\text{)}_5-\text{CH}_3 \\   \\ \text{O}-\text{(CH}_2\text{--CH}_2\text{--O})_p\text{--CO--(CH}_2\text{)}_2\text{--CH}_3 \end{array}$ | 1.0            |
| $\begin{array}{c} \text{CH}-\text{O}-\text{CO}-\text{(CH}_2\text{)}_{10}-\text{CH}-\text{(CH}_2\text{)}_5-\text{CH}_3 \\   \\ \text{O}-\text{(CH}_2\text{--CH}_2\text{--O})_q\text{--CO--(CH}_2\text{)}_2\text{--CH}_3 \end{array}$   |                |
| $\begin{array}{c} \text{CH}_2-\text{O}-\text{CO--(CH}_2\text{)}_{10}-\text{CH}-\text{(CH}_2\text{)}_5-\text{CH}_3 \\   \\ \text{O}-\text{(CH}_2\text{--CH}_2\text{--O})_r\text{--CO--(CH}_2\text{)}_2\text{--CH}_3 \end{array}$       |                |
| Where $p+q+r=150$                                                                                                                                                                                                                     |                |
| Mineral oil (Redwood, viscosity 60 seconds, 30° C.)                                                                                                                                                                                   | 34             |
| Ethylene oxide-higher alcohol adduct nonionic surface active agent + anionic surface active agent                                                                                                                                     | 40             |
|                                                                                                                                                                                                                                       | 25             |

The results in Test 14 (when only component X is used) are undesirable since strength, adhesion and fatigue resistance are all reduced.

Further, in Test 15 (when neither component X nor Y were used and only the mineral oil and the alkyl sulphonate acid salt were used), adhesion is raised, however, both strength and fatigue resistance drop.

### Example 2

A treating agent with the composition shown below was applied to nylon tire cord during the spinning process in a 10 percent aqueous emulsion and in a quantity of 0.5 weight percent to the fiber. After spinning and hot stretching, a 840 denier, 2 ends, 47 filaments per end, tire cord was formed. After treating this cord with the bonding agent as shown in Example No. 1, it was stretched 12 percent at 200° C. for 20 seconds under heat. The results of measurements made of the strength, fatigue resistance and adhesion of the cord were as given in Table 2.

As is evident from the above table, satisfactory results are derived in increasing the strength, the adhesion and the fatigue resistance of the cord that is treated by the method covered in the present invention.

A spinning oil with the composition listed above was applied in a quantity of 0.5 weight percent to nylon 6 tire cord during the spinning process producing improved spinnability. Subsequent to spinning and hot elongation, tire cord similar to that of Example 1 was produced. After treating this cord with the same bonding agent as shown in Example 1, it was heat treated at 200° C., for 20 seconds and a stretch of 12 percent.

35 The results of measuring the strength of the cord, adhesion and fatigue resistance as in Example 1, were as given in Table 3.

TABLE 3

|    |                                                             |                |
|----|-------------------------------------------------------------|----------------|
| 40 | Cord treated by the method covered in the present invention | Degreased cord |
| 45 | Strength of the untreated cord, Kg                          | 15.0           |
|    | Strength of the treated cord, Kg                            | 16.0           |
|    | Adhesion, Kg                                                | 14.0           |
|    | Fatigue resistance, %                                       | 170            |
|    |                                                             | 100            |

TABLE 2

| Composition of the treatment agent                                                                                                                                                                                                | Present invention | Comparative example | Blank      |
|-----------------------------------------------------------------------------------------------------------------------------------------------------------------------------------------------------------------------------------|-------------------|---------------------|------------|
| Partially oxidized polyethylene Y:<br>AC-655 (Allied Chemical Co. mfg.) acid value 15, softening point }<br>104° C., percent.                                                                                                     | 1<br>2.0          | 2<br>2.0            | 3<br>2.0   |
| Nonionic surface active agent:<br>CH <sub>2</sub> —O CO—(CH <sub>2</sub> ) <sub>7</sub> —CH=CH—CH <sub>2</sub> —CH—(CH <sub>2</sub> ) <sub>5</sub> —CH <sub>3</sub><br> <br>O—(CH <sub>2</sub> CH <sub>2</sub> O) <sub>q</sub> —H |                   |                     | 4<br>----- |
| CH—O CO—(CH <sub>2</sub> ) <sub>7</sub> —CH=CH—CH <sub>2</sub> —CH—(CH <sub>2</sub> ) <sub>5</sub> —CH <sub>3</sub><br> <br>O—(CH <sub>2</sub> CH <sub>2</sub> O) <sub>q</sub> —H                                                 | 30.0              |                     | -----      |
| CH <sub>2</sub> —O CO—(CH <sub>2</sub> ) <sub>7</sub> —CH=CH—CH <sub>2</sub> —CH—(CH <sub>2</sub> ) <sub>5</sub> —CH <sub>3</sub><br> <br>O—(CH <sub>2</sub> CH <sub>2</sub> O) <sub>q</sub> —H                                   |                   |                     |            |
| p+q+r=20<br>Polyoxyethylene-(20)-castor oil ester, percent<br>CH <sub>3</sub> —(CH <sub>2</sub> ) <sub>11</sub> —O—(CH <sub>2</sub> CH <sub>2</sub> O) <sub>20</sub> —H                                                           |                   |                     |            |
| Polyoxyethylene-(20)-lauryl ether, percent<br>CH <sub>3</sub> —(CH <sub>2</sub> ) <sub>10</sub> —COO—(CH <sub>2</sub> CH <sub>2</sub> O) <sub>20</sub> —H                                                                         | 30.0              |                     | -----      |
| Polyoxyethylene-(20)-lauryl ester, percent                                                                                                                                                                                        |                   |                     | 30.0       |
| Lubricating agent: Mineral oil (Redwood viscosity 150 sec.), percent                                                                                                                                                              | 50                | 50                  | 50         |
| Ionic surface active agent:<br>Alkyl phosphoric acid ester, percent                                                                                                                                                               | 15                | 15                  | 15         |
| Alkyl sulfonate, percent                                                                                                                                                                                                          | 3                 | 3                   | 3          |
| Properties of the cord:<br>Untreated cord strength, kg.                                                                                                                                                                           | 15.0              | 15.0                | 15.2       |
| Treated cord strength, kg.                                                                                                                                                                                                        | 15.2              | 14.6                | 14.8       |
| Bonding strength, kg.                                                                                                                                                                                                             | 14.0              | 14.0                | 14.2       |
| Fatigue resistance, percent                                                                                                                                                                                                       | 150               | 100                 | 100        |

It was possible to obtain superior results in cord strength, adhesion and resistance to fatigue with the application of the present invention.

Example 4

A treating agent with the composition shown below was applied to nylon tire cord—as the first paragraph of the examples.

Petrolite PE-100, partially oxidized microcrystalline wax,



Commercial Nylon 6 1840 denier as in Example 1, tire cord was washed and degreased, then immersed in a 10 percent trichloroethylene solution to apply 2.0 weight percent of the treating agent. After treatment with the same bonding agent as shown in Practical Example No. 1, it was heat treated for bonding by stretching 12 percent at 200° C. for 20 seconds. The results of measuring the strength, adhesion and fatigue resistance of the cord as described in Example 1, were as given below:

TABLE 4

|                                    | Cord processed by the method covered in the present invention | Degreased cord (blank test) |
|------------------------------------|---------------------------------------------------------------|-----------------------------|
| Strength of the untreated cord, Kg | 15.0                                                          | 14.8                        |
| Strength of the treated cord, Kg   | 15.2                                                          | 14.0                        |
| Adhesion, Kg                       | 14.0                                                          | 11.0                        |
| Resistance to fatigue, %           | 140.0                                                         | 100.0                       |

The strength and the resistance to fatigue of the cord treated by the method covered in the present invention is increased dramatically over that of the untreated cord.

Example 5

A treating agent with the composition shown below was applied to nylon tire cord—as the first paragraph of the examples.

Vp-5001 Hexto Company, oxidized polyethylene, acid value 55



Commercial polyester tire cord (1,000 denier, 2 ends, 50 filaments per end) was washed and degreased, then immersed in a 20 percent aqueous emulsion of the treating agent with 75

the composition shown above to apply 0.7 weight percent to the cord. It was then bonded by stretching 0 percent at 230° C. for 60 seconds. The results of measuring the strength of the cord after treatment were as given in Table 5.

5 The bonding agent used during the bonding treatment was the bonding compound shown in Example 1, to which 5 weight percent of Epicoat 812<sup>4</sup> was added. This compound was applied in an amount equal to 8 percent of the fiber.

Percent weight

2.0

13.0  
85.0

TABLE 5

|                                                                | Strength prior to bonding treatment | Strength after bonding treatment |
|----------------------------------------------------------------|-------------------------------------|----------------------------------|
| 30 Cord treated by the method covered in the present invention | 14.7 Kg                             | 14.3 Kg                          |
| 35 Degreased cord (comparative example)                        | 14.7 Kg                             | 13.0 Kg                          |
| Commercial cord (comparative example)                          | 14.9 Kg                             | 13.8 Kg                          |

40

45

Example 6

A treating agent with the composition shown below was applied during the spinning of nylon tire cord. 10 percent aqueous emulsions in which the molar numbers ( $p+q+r$ ) of ethylene oxide added to a polyoxyethylene castor oil ester were varied, were applied to the cord in amounts equivalent to 0.5 weight percent. The cord was hot stretched to form a 840 denier, 2 ends, 47 filaments per end, tire cord. After treating this cord with a bonding agent similar to that described in Example 1, it was hot stretched 12 percent at 200° C. for 20 seconds. The results of measuring the strength, resistance to

Percent weight

2.5

34.5  
40.0  
23.0

fatigue and adhesions of the cord were as given in Table 6.  
Composition of the treating agent.  
Polyoxyethylene castor oil ester.

Percent



4. Glycerol di-glycidyl ether,  
Epolene E, Eastman Company, partially oxidized polyethylene, acid value 12,  
softening point 97° C.  
Mineral oil (Redwood viscosity 60 seconds)  
Alkyl phosphoric acid ester

0.1  
30.0  
29.9

| Molar number for the ethylene oxide added $p+q+r$ | Comparative |      |      |      |      |      | Comparative example |      |       |
|---------------------------------------------------|-------------|------|------|------|------|------|---------------------|------|-------|
|                                                   | 4           | 5    | 10   | 24   | 40   | 100  | 300                 | 305  | Blank |
| Strength of the untreated cord, kg                | 15.1        | 15.1 | 15.1 | 15.0 | 15.0 | 15.0 | 15.0                | 15.0 | 15.0  |
| Strength of the treated cord, kg                  | 15.2        | 15.3 | 15.2 | 15.2 | 15.2 | 15.2 | 15.0                | 14.0 | 14.0  |
| Adhesion, kg                                      | 15.0        | 15.8 | 14.0 | 14.0 | 14.0 | 14.2 | 14.3                | 14.4 | 11.0  |
| Fatigue resistance, percent                       | 131         | 130  | 130  | 130  | 130  | 130  | 120                 | 115  | 100   |

As is clear from the above table the strength, adhesion and fatigue strength of the treated cord with the molar numbers,  $p+q+r$  of the ethylene oxide added within the limits of 5 to 300 as in the method covered by the present invention were superior. Conversely, when the molar numbers of the ethylene oxide added were low ( $p+q+r=4$ ), the strength and fatigue resistance raised but adhesion was insufficient.

Further, when the molar numbers of the ethylene oxide added were high ( $p+q+r=305$ ) no treatment effects appeared owing to difficulty in emulsification, adhesion was improved. However, no improvement in strength was observed and there was little increase in fatigue resistance.

I CLAIM:

1. A method for the treatment of synthetic fibers used for reinforcing rubber comprising applying a thin coating of a treating agent to said fibers, said treating agent comprising

a. 5 to 40 percent by weight of the said treating agent of a nonionic surface active agent having the following general formula:



where  $\Lambda$  represents  $(\text{CH}_2)_7$ ,  $\text{CH} = \text{CH-CH}_2$  or  $(\text{CH}_2)_{10}$ ;  $\text{R}_1$ ,  $\text{R}_2$  and  $\text{R}_3$  represent hydrogen atoms  $-\text{CO-R}'_1$ ,  $-\text{CO-R}'_2$ , or  $-\text{CO-R}'_3$ ; and  $\text{R}'_1$ ,  $\text{R}'_2$  and  $\text{R}'_3$  represent aliphatic hydrocarbons with carbon numbers of 1 to 22,  $p$ ,  $q$ , and  $r$  represent the molar numbers of the ethylene oxide added and  $p+q+r$  is a positive integer = 5 to 300,

2. 0.1 to 3.0 percent by weight of the said treating agent of partially oxidized polyethylene with an average molecular weight of 500 to 10,000,

3. the remaining percent by weight of the said treating agent of a lubricating agent for said fibers and an ionic surface active agent or a nonionic surface active agent which is different from the nonionic surface active agent in (a).

25 4. The method of claim 1 wherein the synthetic fiber is selected from the group consisting of nylon and polyester, the coating is applied to achieve 0.01 to 2.0 percent by weight of the fiber, the partially oxidized polyethylene has an acid value of 10 to 30 and a softening point below 125° C., the lubricating agent is a mineral oil, a higher aliphatic alcohol ester, or a vegetable oil, and the second surface active agent is a higher alcohol-ethylene oxide adduct, a sulfuric acid ester salt, or a phosphoric acid ester salt.

30 5. The method of claim 2 wherein the nylon is nylon 6, and  $\text{R}'_1$ ,  $\text{R}'_2$  and  $\text{R}'_3$  have carbon numbers of 8 to 17.

35 6. The method of claim 2 wherein the polyester is polyethylene terephthalate, and  $\text{R}'_1$ ,  $\text{R}'_2$  and  $\text{R}'_3$  have carbon numbers of 8 to 17.

\* \* \* \* \*

55

60

65

70

75